# EUROPEAN PATENT SPECIFICATION

(11) **EP 2 925 847 B1**
(45) Date of publication and mention of the grant of the patent: **27.07.2016**
(21) Application number: 13795253.7
(22) Date of filing: 25.11.2013
(51) Int. Cl.: C11D 3/37, C11D 1/02

(54) **THICKENED AQUEOUS DETERGENT LIQUID**
ANGEDICKTE WÄSSRIGE REINIGUNGSFLÜSSIGKEIT
LIQUIDE DÉTERGENT AQUEUX ÉPAISSI

(30) Priority: 29.11.2012 WO PCT/CN2012/085567
(43) Date of publication of application: 07.10.2015
(73) Proprietor: Unilever PLC, London, Greater London EC4Y 0DY (GB); Unilever N.V., 3013 AL Rotterdam (NL)
(72) Inventor: JARVIS, Adam, Peter, Bebington Wirral Merseyside CH63 3JW (GB); LIMER, Adam, John, Shanghai200335 (CN); RYAN, Philip, Michael, Bebington Wirral Merseyside CH63 3JW (GB); THOMAS, Matthew, Rhys, Bebington Wirral Merseyside CH63 3JW (GB)
(74) Representative: Newbould, Frazer Anthony
(86) International application number: PCT/EP2013/074596
(87) International publication number: WO 2014/082955

(56) References cited:
- EP-A1- 0 896 027
- EP-A1- 1 721 915
- EP-A2- 0 248 612
- WO-A1-2008/017620
- US-A- 4 384 096
- US-A- 5 057 241

## Description

### TECHNICAL FIELD

This invention relates to aqueous detergent compositions comprising an alkali swellable acrylic based rheology modifying polymer emulsion with hydrophobic modification, or HASE polymer.

### BACKGROUND

A trend in detergent formulating is to reduce the amount of surfactant and to replace these petrochemical derived ingredients with highly weight efficient ingredients selected from cleaning and soil release polymers, sequestrants and enzyme cocktails. Typically some surfactant is retained in the composition and the work horse surfactant linear alkyl benzene sulphonate (LAS) is frequently a key part of the surfactant blend. The polymer ethoxylated polyethylene imine may be used as one of the weight efficient ingredients. Suitable compositions are taught, for example, in WO09153184.

It has been found that consumers prefer that the new type of concentrated liquid is thickened so that it conveys the impression of high contents when in the bottle. On the other hand it is desirable that the pour viscosity is low enough that dosing can be done easily and accurately. A shear thinning composition is thus desired.

Hydrophobically modified alkali swellable emulsion (HASE) copolymers are a type of synthetic associative thickener. This thickener typically contains a backbone consisting of randomly distributed methacrylic acid (MAA) and ethylacrylate (EA) monomers.

Inserted into this backbone are a small proportion of hydrophobically modified groups, usually less than 3 mol%. The monomers to form these hydrophobic groups are sometimes referred to as surfmers or associative monomers. Due to its structure, the copolymer, when dissolved in an alkaline aqueous liquid, induces a variety of interacting forces such as hydrophobic, hydrogen bonding, electrostatic, etc and this modifies the rheology of the liquid.

HASE copolymers are usually synthesized via the emulsion polymerization technique.

US 5 015 711 (Coatex) discloses a thickening terpolymer of the MAA/EA/surfmer type. US 5 015 711 makes the following disclosure: "The first type of monomer, which is a carboxylic acid with an ethylenic unsaturation site, is a C₃-C₂₀, preferably C₃-C₁₂, compound having an ethylenic bond and at least one carboxylic group or a carboxylic acid anhydride group. The carboxylated ethylenic monomer can be selected from among monoacids, such as acrylic acid, methacrylic acid, crotonic acid, isocrotonic acid, cinnamic acid, diacids, such as itaconic acid, fumaric acid, maleic acid, and citraconic acid, carboxylic acid anhydrides, such as maleic anhydride and diacid hemiesters, such as the C₁₋₄ monoesters of maleic or itaconic acids. However, the carboxyl ethylene monomer is preferably selected from the group consisting of acrylic acid, methacrylic acid and itaconic acid".

US 4 384 096 discloses a copolymer having 42% MAA, 6% IA, 42%EA and 10% surfmer (where IA is itaconic acid). The surfmer used was Nonylphenoxy poly(ethyleneoxy)₉ ethyl Methacrylate. US 4 384 096 contains a general disclosure relating to the use of Itaconic acid as follows: "Acrylic or methacrylic acid or a mixture thereof with itaconic or fumaric acid are preferred, but crotonic and aconitic acid and half esters of these and other polycarboxylic acids such as maleic acid with C₁ - C₄ alkanols are also suitable, particularly if used in minor amount in combination with acrylic or methacrylic acid". The itaconic acid containing polymer was not tested for its pH response.

Thickened pseudoplastic detergent compositions are also known from US5057241.

The manufacture of LAS-containing liquid detergent compositions, for example compositions intended for laundry or hard surface cleaning applications, typically entails the neutralisation of the corresponding alkylbenzene sulphonic acid with base. During the manufacturing process a very high pH composition may temporarily be formed. We have found that when some HASE polymers are exposed to a pH above about 10 they may no longer function efficiently. The detergent formulator would like to be able to have freedom to use manufacturing processes where the pH may temporarily rise above 10. It is thus an objective to find thickening polymer that can be neutralised along with the surfactant and which can function efficiently even if it is temporarily exposed to a pH of more than 10 during processing.

### SUMMARY OF THE INVENTION

According to the present invention there is provided a thickened aqueous detergent liquid comprising:
(i) at least 5 wt% of a surfactant system comprising anionic surfactant,
(ii) at least 0.2 wt% of a thickening system comprising a linear copolymer formed by the addition polymerisation of:
   (A) 0.1 to 5 wt% of a first monomer consisting of an ethylenically unsaturated diacid of formula (I):

      HOOC-CR₁=CR₂-COOH (I)

      or an unsaturated cyclic anhydride precursor of such an ethylenically unsaturated diacid, the anhydride having formula (II) where R₁ and R₂ are individually selected from H, C₁-C₃ alkyl, phenyl, chlorine and bromine;
   (B) 15 to 60 wt% of a second ethylenically unsaturated monoacidic monomer consisting of (meth)acrylic acid;
   (C) 30 to 70 wt% of a third ethylenically unsaturated monomer consisting of C₁-C₈ alkyl ester of (meth)acrylic acid; and
   (D) 1 to 25 wt%, of a fourth ethylenically unsaturated monomer, consisting of surfmer of formula (III):
      wherein each R₃ and R₄ are each independently selected from H, methyl, - C(=O)OH, or -C(=O)OR₅;
      R₅ is a C₁-C₃₀ alkyl;
      T is -CH₂C(=O)O-, -C(=O)O-, -O-, -CH₂O-, -NHC(=O)NH-, -C(=O)NH-, -Ar-(CE₂)_{z}-NHC(=O)O-, -Ar-(CE₂)_{z}-NHC(=O)NH-, or -CH₂CH₂NHC(=O)-;
      Ar is divalent aryl;
      E is H or methyl;
      z is 0 or 1;
      k is an integer in the range of 0 to 30; and m is 0 or 1; with the proviso that when k is 0, m is 0, and when k is in the range of 1 to 30; m is 1;
      (R₆O)ₙ is polyoxyalkylene, which is a homopolymer, a random copolymer, or a block copolymer of C₂-C₄-oxyalkylene units, wherein R₆ is C₂H₄, C₃H₆, C₄H₈, or a mixture thereof, and n is an integer in the range of 5 to 250;Y is -R₆O-,-R₆-, -C(=O)-, -C(=O)NH-, =R₆NHC(=O)NH-, or -C(=O)NHC(=O)-; and
      R₇ is substituted or unsubstituted alkyl selected from the group consisting of C₈-C₄₀ linear alkyl, C₈-C₄₀ branched alkyl, C₈-C₄₀ carbocyclic alkyl, C₂-C₄₀ alkyl-substituted, phenyl, aryl-substituted C₂-C₄₀ alkyl, and C₈-C₈₀ complex ester; wherein the R₇ alkyl group optionally comprises one or more substituents selected from the group consisting of hydroxy, alkoxy, and halogen.

Preferably Surfmer D has the formula (IV) where:
R₈ and R₉ are each independently selected from H, and C₁₋₃ alkyl;
R₁₀ is C₂-C₄ and mixtures thereof, preferably C₂;
m, the average number of alkoxy units R₁₀O, is from 6 to 40;
R₁₁ is alkyl or alkylaryl where the alkyl part is linear or branched; and
the total number of carbons is from 10 to 40.

In this specification the term (meth)acrylic acid includes both acrylic acid and methacrylic acid and the term (meth)acrylate includes both acrylate and methacrylate.

The viscosity of the liquid at 20 s⁻¹ and 25°C is preferably at least 0.3 Pa.s, most preferably at least 0.4 Pa.s.

The compositions preferably comprise at least 1 wt% of the copolymer (ii).

Copolymer (ii) preferably has a molecular weight Mw of over 250 000, more preferably over 500 000 Daltons.

The copolymers (ii) are linear, that is uncrosslinked, alkali swellable hydrophobically modified acrylic copolymers, HASE. These polymers require alkaline conditions to swell and so should be added to the composition such that they are exposed to alkaline conditions at some stage during the manufacture of the detergent liquid.

In order to provide maximum charge density and improved swelling it is preferred to use maleic acid as the diacid (A) in copolymer (ii). Conveniently maleic anhydride is used as the first monomer A in the copolymerisation.

Also according to the invention there is provided a process for manufacture of a detergent composition, the process comprising mixing a linear HASE copolymer formed from Monomers A, B C and D as described above with an acid precursor of an anionic surfactant and then adding alkali sufficient to neutralise the surfactant acid and to swell the copolymer.

### DETAILED DESCRIPTION OF THE INVENTION

### First Monomer A

The copolymer is formed using a monomer A which may ring open to form a diacidic unit in the polymer. Diacidic unit means that carboxylate groups are attached to adjacent carbon atoms in the carbon backbone of the copolymer. Conveniently this unit is formed from a cyclic ethylenically unsaturated anhydride monomer of formula (II). It is preferred that monomer A is such an anhydride. where R₁ and R₂ are individually selected from H, C₁-C₃ alkyl, phenyl, chlorine and bromine. Use of a cyclic anhydride monomer with ethylenic unsaturation gives a cis diacid if the ring opens. Such a diacid has both carboxylate groups arranged on the same side of the polymer - but on different carbon atoms.

Preferably R₁ is hydrogen and R₂ is selected from the group comprising hydrogen, methyl, bromine and phenyl. More preferably R₁ is hydrogen and R₂ is selected from hydrogen and methyl. Most preferably R₁ and R₂ are hydrogen so that the anhydride is maleic anhydride. This is the precursor for maleic acid. It is thought that because maleic acid produces carboxylate groups on adjacent carbon atoms in the polymer backbone this increases the localised charge density and causes the difference in performance compared with copolymers not containing this diacid. Itaconic acid which is outside the scope of this invention provides a polymer element where one carbon carries two carboxylate groups and the other carries none. Fumaric acid is the trans isomer of maleic acid it cannot be formed from maleic anhydride monomer by hydrolysis during the emulsion polymerization.

Monomer A may range from 0.1 to 5 wt%, preferably from 0.2 to 4 wt%, and more preferably from 0.3 to 1 wt%, and optimally from 0.4 to 0.6 wt% of the total copolymer.

### Second Monomer B

The second monomer B is a monoacidic vinyl monomer. Suitable monomers are acrylic acid, methacrylic acid, salts of the aforementioned acids and combinations thereof.

In the compositions, the acid groups may be neutralized to form salts. Typical salt counterions to the acid groups are sodium, potassium, ammonium and triethanolammonium cations.

Amounts of the monoacidic vinyl monomer in the copolymers may range from 15 to 60 wt%, preferably from 20 to 55 wt%, more preferably from 25 to 50 wt% of the total copolymer.

### Third Monomer C

The third monomer, C, includes one or more C₁-C₈ esters of acrylic or methacrylic acid. Illustrative ester monomers are ethylacrylate, methylacrylate, ethylmethacrylate, methylmethacrylate, butylacrylate, butylmethacrylate and mixtures thereof. Ethyl acrylate is most preferred.

The amount of acrylate ester monomers in the copolymer may range from 30 to 70 wt%, preferably from 25 to 60 wt%, and more preferably from 40 to 65 wt% of the total copolymer.

### Fourth Monomer D

The fourth ethylenically unsaturated monomer, consists of a surfmer of formula (III): wherein
R₃ and R₄ are each independently selected from H, methyl, -C(=O)OH, or-C(=O)OR₅; and R₅ is a C₁-C₃₀ alkyl;
T is -CH₂C(=O)O-, -C(=O)O-, -O-, -CH₂O-, -NHC(=O)NH-, -C(=O)NH-, -Ar-(CE₂)_{z}-NHC(=O)O-, -Ar-(CE₂)_{z}-NHC(=O)NH-, or -CH₂CH₂NHC(=O)-;
Ar is divalent aryl;
E is H or methyl;
z is O or 1;
k is an integer in the range of 0 to 30; and m is 0 or 1;
with the proviso that when k is 0, m is 0, and when k is in the range of 1 to 30; m is 1;
(R₆O)ₙ is polyoxyalkylene, which is a homopolymer, a random copolymer, or a block copolymer of C₂-C₄-oxyalkylene units, wherein R₆ is C₂H₄, C₃H₆, C₄H₈,
or a mixture thereof, and n is an integer in the range of 5 to 250;Y is -R₂O-,-R₆-, -C(=O)-, -C(=O)NH-, =R₆NHC(=O)NH-, or-C(=O)NHC(=O)-; and
R₇ is substituted or unsubstituted alkyl selected from the group consisting of C₈-C₄₀ linear alkyl, C₈-C₄₀ branched alkyl, C₈-C₄₀ carbocyclic alkyl, C₂-C₄₀ alkyl-substituted, phenyl, aryl-substituted C₂-C₄₀ alkyl, and C₈-C₈₀ complex ester; wherein the R₇ group optionally comprises one or more substituents selected from the group consisting of hydroxy, alkoxy, and halogen.

Preferably Surfmer D has the formula (IV) where:
R₈ and R₉ are each independently selected from H, and C₁₋₃ alkyl;
R₁₀ is C₂-C₄ and mixtures thereof, preferably C₂;
m, the average number of alkoxy units R₁₀O, is from 6 to 40;
R₁₁ is alkyl or alkylaryl where the alkyl part is linear or branched; and the total number of carbons is from 10 to 40.

The fourth monomer D is more preferably a surfmer of formula (V). in which each R₈ and R₉ are independently selected from H, C₁ to C₃ alkyl

Preferably R₈ is a methyl group and R₉ is H. n ranges from 6 to 40 and m ranges from 6 to 40, preferably n ranges from 10 to 30 and m ranges 15 to 35 most preferably n ranges from 12 to 22 and m ranges from 20 to 30. It is preferable that m is greater or equal to n.

The amount of surfmer D in the copolymer may range from 1 to 25 wt%, preferably from 3 to 20 wt%, and more preferably from 2 to a 12 wt% of the total copolymer.

Preferably the level of copolymer in the thickening system is from 0.2 to 3 wt% of the total composition; more preferably from 0.4 to 2 wt%, even 0.5 to 2 wt%

The copolymers may be used with other thickeners to make up the thickening system. Preferred co-thickeners are other thickening polymers and thickening clays.

Preferably the surfactant system comprises at least 3 wt% of anionic surfactant, most preferably the anionic surfactant comprises linear alkyl benzene sulphonate.

Advantageously the composition comprises one or more further polymers that are included in the composition for purposes other than rheology modification. Such further polymers may reduce the viscosity of the compositions and this reduction can be compensated for by the inclusion of the thickening polymer. Preferred further polymers are ethoxylated polyethylene imine and/or polyester soil release polymer. Both of these polymers have been found to thin the detergent compositions. Preferably the detergent liquid further comprises at least 1 wt% ethoxylated polyethylene imine polymer. Most preferably it further comprises at least 0.5 wt% of polyester soil release polymers. More preferably the composition comprises at least 3 wt% of ethoxylated polyethylene imine.

Advantageously the detergent composition comprises an effective amount of at least one enzyme selected from the group comprising, pectate lyase, protease, amylase, cellulase, lipase, mannanase. More advantageously it comprises at least 2 of this group of enzymes even more advantageously at least 3 and most advantageously at least 4 of the enzymes from this group.

The invention will now be further described with reference to the following nonlimiting examples and to the drawings which are briefly described as:
Figure 1 - is a graph showing viscosity changes with pH for Carbopol 980 (a prior art ASE copolymer);
Figure 2 - is a graph showing viscosity changes with pH for Acusol 820 (a prior art HASE copolymer);
Figure 3 - is a graph showing viscosity changes with pH for a linear HASE Copolymer made using a maleic anhydride monomer; and
Figure 4 - is a graph showing viscosity changes with pH for a further linear HASE copolymer made using a maleic anhydride monomer.

### EXAMPLES

### Surfmer Synthesis

n = 12
m = 23

Brij® 35P (150 g) from Sigma Aldrich was dissolved in 500 ml anhydrous dichloromethane under a nitrogen atmosphere and cooled in an ice bath to 5 °C. Triethylamine (18.6 g) was added via syringe before methacryloyl chloride (20.9 g) was added dropwise over a 30 minute period. After complete addition, the solution was allowed to warm to room temperature and the reaction stirred for 4 weeks. The solution was then filtered to remove the resulting precipitate and washed once with saturated sodium hydrogen carbonate solution (200 ml) and once with saturated brine (200 ml). The solution was then passed through a column containing basic alumina before the product was dried with anhydrous magnesium sulphate, filtered and the solvent removed in vacuo. In subsequent examples the product is referred to as Surfmer A.

### HASE copolymer synthesis

A round bottom flask was charged with ethyl acrylate (EA) (66.8 g), methacrylic acid (MAA) (37.7 g), maleic anhydride (MA) (0.515 g) and Surfmer A (10.0 g). The mixture was sealed and purged with nitrogen for 60 minutes before sodium dodecyl sulfonate (1.03 g) and deoxygenated water (26.5 g) was added and stirred forming a pre-emulsion. A multineck round bottom flask was fitted with a nitrogen sparge and overhead stirrer. Deoxygenated water (181 g) and sodium dodecyl sulfonate (0.298 g) were added, stirred at 250 rpm and heated to 90 °C. Ammonium persulfate (0.073 g) in water (1 ml) was added via syringe. The pre-emulsion was fed into the surfactant solution via peristaltic pump over 150 minutes. After complete addition, ammonium persulfate (0.033 g) in water (1 ml) was added and the reaction stirred for a further 240 minutes. The resulting product is hereafter referred to as Copolymer 1. Further Copolymers 2, and 3 were synthesised by using suitable adaptations of this process. All the Copolymers are detailed in Table 1.

**Table 1**

| Polymer | MAA | MA | EA | Surfmer A |
|---|---|---|---|---|
| 1 | 32.8 | 0.45 | 58.1 | 8.7 |
| 2 | 34.6 | 0.47 | 61.4 | 3.5 |
| 3 | 35.2 | 0.58 | 57.7 | 6.5 |

### pH testing

Figures 1 and 2 show how for various known associative thickening polymers the viscosity drops off again at high pH.

Figure 1 is Carbopol 980 a crosslinked hydrophobically modified (surfmer containing) MMA copolymer. The Copolymer was added to water at 2.9 wt% and then neutralised with NaOH. Allowing time for swelling to occur each time before testing the viscosity of a sample of the thickened liquid using an Anton Paar viscometer. Adding further acid to reduce the pH once the thinning effect commenced at high pH did not increase the viscosity.

Figure 2 shows another very similar viscosity fall off for a linear hydrophobically modified acrylate copolymer sold by Dow as Acusol 820. The copolymer was added to water at 0.8 wt%, neutralised with NaOH and tested in the same way as for the Carbopol.

Figures 3 shows the same test done with linear copolymer 1 used at 2.8 wt% and neutralised with NaOH. Figure 4 shows the same test done with 1 wt% copolymer 3. The reduction of viscosity once a threshold pH is exceeded is not seen for these copolymers made with maleic anhydride.

### Liquid compositions using the Copolymers

The alkalinity resistant copolymers give flexibility to the detergent formulator to use manufacturing processes that may expose the copolymers to high pH without fear of loss of rheology as a consequence. They are thus especially useful for compositions which contain anionic surfactants that are normally neutralised during the manufacture of the detergent liquid; thus allowing the heat evolved to be used for assisting with incorporation of other ingredients into the compositions, especially nonionic surfactants.

To test the resilience of the polymer to being added prior to neutralisation of the surfactant acid the aqueous detergent liquid given in Table 2 was made. In this example the polymer is mixed with some of the alkali and the acid added to this mixture before the remainder of the alkali is added. The order of addition of the key ingredients is shown, the remaining ingredients are added once the key ingredients have been mixed and neutralised.

**Table 2**

| Ingredient | Level (wt%) as 100% active | Order of addition |
|---|---|---|
| Water | 37.7 | 1 |
| Fluorescer | 0.25 | 2 |
| MPG | 8.0 | 3 |
| Nonionic surfactant | 8.4 | 4 |
| Copolymer 3 | 1.0 | 5 |
| Alkaline Neutraliser (MEA) | 6.2 | 6 |
| Anionic surfactant acid (LAS) | 11.2 | 7 |
| Alkaline Neutraliser (TEA) | 4.0 | 8 |
| Citric acid | 2.5 | |
| Fatty acid | 3.5 | |
| Sequestrant | 1.5 | |
| Anti oxidant | 0.25 | |
| Pre-neutralised Anionic surfactant (SLES) | 8.4 | |
| EPEI | 3.0 | |
| Perfume | 1.4 | |
| Opacifier | 0.1 | |
| Enzymes | 2.6 | |

After 8 weeks on store the thickened detergent liquid so produced is still homogeneous and has the following viscosity profile at room temperature shown in Table 3.

**Table 3**

| Shear rate | Viscosity (mPa.s) |
|---|---|
| 2 s⁻¹ | 389 |
| 21 s⁻¹ | 341 |
| 106 s⁻¹ | 308 |

Some further suitable liquid detergent formulations are given in Table 4 below.

**Table 4 - Exemplary detergent compositions**

| Liquid | A | B |
|---|---|---|
| Water | 58.8 | 58.5 |
| LAS | 7.8 | 9.2 |
| SLES | 2.9 | 4.6 |
| Nonionic | 5.5 | 14.0 |
| Fatty acid | 4.5 | 1.5 |
| Alkaline Neutraliser | 8.3 | 2.9 |
| Glycerol | 7.5 | 5.0 |
| MPG | 0.0 | 2.0 |
| Sequestrant | 3.6 | 0.3 |
| HASE copolymer | 0.8 | 0.1 |
| Soil release polymer | 0.1 | 0.0 |
| Enzymes | 0.0 | 0.8 |
| Perfume, colorant and opacifier | 0.6 | 1.5 |
| Fluorescer | 0.0 | 0.1 |
| Preservative and antioxidant | 0.3 | 0.0 |
| NB - above inclusion levels are all as 100% active | | |

LAS is linear alkyl benzene sulphonic acid
SLES is sodium lauryl ether sulphate 3EO
EPEI is ethoxylated polyethylene imine PEI(600) 20EO
MPG is Monopropylene glycol
HASE copolymer is Copolymer 1,2 or 3

## Claims

1. A thickened aqueous detergent liquid comprising:
(i) at least 5 wt% of a surfactant system comprising anionic surfactant,
(ii) at least 0.2 wt% of a thickening system comprising a linear copolymer formed by the addition polymerisation of:
(A) 0.1 to 5 wt% of a first monomer consisting of an ethylenically unsaturated diacid of formula (I):
HOOC-CR₁=CR₂-COOH (I)
or an unsaturated cyclic anhydride precursor of such an ethylenically unsaturated diacid, the anhydride having formula (II) where R₁ and R₂ are individually selected from H, C₁-C₃ alkyl, phenyl, chlorine and bromine;
(B) 15 to 60 wt% of a second ethylenically unsaturated monoacidic monomer consisting of (meth)acrylic acid;
(C) 30 to 70 wt% of a third ethylenically unsaturated monomer consisting of C₁-C₈ alkyl ester of (meth)acrylic acid;
(D) 1 to 25 wt%, of a fourth ethylenically unsaturated monomer, consisting of surfmer of formula (III):
wherein each R₃ and R₄ are each independently selected from H, methyl, -C(=O)OH, or -C(=O)OR₅;
R₅ is a C₁-C₃₀ alkyl;
T is -CH₂C(=O)O-, -C(=O)O-, -O-, -CH₂O-, -NHC(=O)NH-, -C(=O)NH-, -Ar-(CE₂)_{z}-NHC(=O)O-, -Ar-(CE₂)_{z}-NHC(=O)NH- or -CH₂CH₂NHC(=O)-;
Ar is divalent aryl;
E is H or methyl;
z is 0 or 1;
k is an integer in the range of 0 to 30; and m is 0 or 1; with the proviso that when k is 0, m is 0, and when k is in the range of 1 to 30; m is 1;
(R₆O)ₙ is polyoxyalkylene, which is a homopolymer, a random copolymer, or a block copolymer of C₂-C₄-oxyalkylene units, wherein R₆ is C₂H₄, C₃H₆, C₄H₈, or a mixture thereof, and n is an integer in the range of 5 to 250;Y is -R₆O-, -R₆-, -C(=O)-, -C(=O)NH-, =R₆NHC(=O)NH-, or -C(=O)NHC(=O)-; and
R₇ is substituted or unsubstituted alkyl selected from the group consisting of C₈-C₄₀ linear alkyl, C₈-C₄₀ branched alkyl, C₈-C₄₀ carbocyclic alkyl, C₂-C₄₀ alkyl-substituted, phenyl, aryl-substituted C₂-C₄₀ alkyl, and C₈-C₈₀ complex ester; wherein the R₇ alkyl group optionally comprises one or more substituents selected from the group consisting of hydroxy, alkoxy, and halogen.

2. A composition according to claim 1 wherein fourth monomer D is a Surfmer with formula (IV): where:
R₈ and R₉ are each independently selected from H, and C₁₋₃ alkyl;
R₁₀ is C₂-C₄ and mixtures thereof, preferably C₂;
m, the average number of alkoxy units R₁₀O, is from 6 to 40;
R₁₁ is alkyl or alkylaryl where the alkyl part is linear or branched; and
the total number of carbons is from 10 to 40.

3. A composition according to any preceding claim wherein the fourth monomer D is a Surfmer with formula (V): in which each R₈ and R₉ are independently selected from H, C₁ to C₃ alkyl, preferably R₈ is a methyl group and R₉ is H, n ranges from 6 to 40 and m ranges from 6 to 40, preferably n ranges from 10 to 30 and m ranges 15 to 35 most preferably n ranges from 12 to 22 and m ranges from 20 to 30.

4. A composition according to any preceding claim wherein the viscosity of the liquid at 20 s⁻¹ and 25°C is at least 0.3 Pa.s, preferably at least 0.4 Pa.s.

5. A composition according to any preceding claim comprising at least 0.4 wt% of the copolymer (ii).

6. A composition according to any preceding claim wherein the anionic surfactant is selected from the group consisting of alkyl benzene sulphonate, and alkyl sulphate.

7. A composition according to any preceding claim wherein the anionic surfactant comprises linear alkyl benzene sulphonate, sodium salt.

8. A composition according to any preceding claim wherein the composition further includes a viscosity reducing polymer selected from ethoxylated polyethylene imine and polyester soil release polymer.

9. A composition according to any preceding claim wherein the copolymer (ii) has a molecular weight Mw of at least 500,000 Daltons.

10. A composition according to any preceding claim in which the first monomer (A) in copolymer (ii) is maleic anhydride.

11. A process for manufacture of a detergent composition, the process comprising mixing a linear HASE copolymer formed from Monomers A, B C and D as described above with an acid precursor of an anionic surfactant and then adding alkali sufficient to neutralise the surfactant acid and to swell the copolymer.

## Patentansprüche

1. Eine verdickte wässrige Reinigungsmittelflüssigkeit, umfassend:
(i) mindestens 5 Gew.-% eines Tensidsystems, umfassend anionisches Tensid,
(ii) mindestens 0,2 Gew.-% eines Verdickersystems, umfassend ein lineares Copolymer, gebildet durch Additionspolymerisation von:
(A) 0,1 bis 5 Gew.-% eines ersten Monomers, bestehend aus einer ethylenisch ungesättigten Disäure der Formel (I):
HOOC-CR₁=CR₂-COOH (I)
oder eines ungesättigten cyclischen Anhydridvorläufers einer solchen ethylenisch ungesättigten Disäure, wobei das Anhydrid die Formel (II) aufweist wobei R₁ und R₂ unabhängig ausgewählt sind aus H, C₁-C₃-Alkyl, Phenyl, Chlor und Brom;
(B) 15 bis 60 Gew.-% eines zweiten ethylenisch ungesättigten Monosäuremonomers, bestehend aus (Meth)acrylsäure;
(C) 30 bis 70 Gew.-% eines dritten ethylenisch ungesättigten Monomers, bestehend aus C₁-C₈-Alkylester von (Meth)acrylsäure;
(D) 1 bis 25 Gew.-% eines vierten ethylenisch ungesättigten Monomers, bestehend aus Surfmer der Formel (III):
wobei jedes R₃ und R₄, unabhängig voneinander, ausgewählt ist aus H, Methyl, -C(=O)OH oder -C(=O)OR₅;
R₅ ein C₁-C₃₀-Alkylrest ist;
T -CH₂C(=O)O-, -C(=O)O-, -O-, -CH₂O-, -NHC(=O)NH-, -C(=O)NH-, - Ar-(CE₂)_{z}-NHC(=O)O-, -Ar-(CE₂)_{z}-NHC(=O)NH- oder -CH₂CH₂NHC(=O)-ist;
Ar ein divalenter Arylrest ist;
E H oder Methyl ist;
z 0 oder 1 ist;
k ein ganze Zahl im Bereich von 0 bis 30 ist; und m 0 oder 1 ist; mit der Maßgabe, dass wenn k 0 ist, m 0 ist und wenn k im Bereich von 1 bis 30 ist, m 1 ist;
(R₆O)ₙ Polyoxyalkylen ist, das ein Homopolymer, ein statistisches Copolymer oder ein Blockcopolymer von C₂-C₄-Oxyalkyleneinheiten ist, wobei R₆ C₂H₄, C₃H₆, C₄H₈ oder eine Mischung davon ist und n eine ganze Zahl im Bereich von 5 bis 250 ist; Y -R₆O-, -R₆-, -C(=O)-,-C(=O)NH-, =R₆NHC(=O)NH- oder -C(=O)NHC(=O)- ist und
R₇ ein substituierter oder unsubstituierter Alkylrest, ausgewählt aus der Gruppe, bestehend aus C₈-C₄₀ linearem Alkylrest, C₈-C₄₀ verzweigtem Alkylrest, C₈-C₄₀ carbocyclischem Alkylrest, C₂-C₄₀-substituiertem Alkylrest, Phenyl, Aryl-substituiertem C₂-C₄₀-Alkylrest, und C₈-C₈₀ Komplexester ist, wobei die R₇-Alkylgruppe optional einen oder mehrere Substituenten, ausgewählt aus der Gruppe, bestehend aus Hydroxy, Alkoxy und Halogen, aufweist.

2. Eine Zusammensetzung gemäß Anspruch 1, wobei das vierte Monomer D ein Surfmer der Formel (IV) ist:
wobei R₈ und R₉ jeweils unabhängig ausgewählt sind aus H und C₁-₃-Alkylrest;
R₁₀ C₂-C₄ und Mischungen davon, vorzugsweise C₂, ist;
m, die gemittelte Anzahl der Alkoxyeinheiten R₁₀O, von 6 bis 40 ist;
R₁₁ Alkyl oder Alkylaryl ist, wobei der Alkylteil linear oder verzweigt ist; und die Gesamtanzahl von Kohlenstoffatomen von 10 bis 40 ist.

3. Eine Zusammensetzung gemäß jedem der vorstehenden Ansprüche, wobei das vierte Monomer D ein Surfmer mit der Formel (V) ist: in der jedes R₈ und R₉ unabhängig ausgewählt sind aus H, C₁-C₃-Alkyl, vorzugsweise R₈ eine Methylgruppe ist und R₉ H ist, n von 6 bis 40 reicht und m von 6 bis 40 reicht, vorzugsweise n von 10 bis 30 reicht und m von 15 bis 35 reicht, und meist bevorzugt n von 12 bis 22 und m von 20 bis 30 reicht.

4. Eine Zusammensetzung nach irgendeinem der vorstehenden Ansprüche, wobei die Viskosität der Flüssigkeit bei 20 s⁻¹ und 25°C mindestens 0,3 Pa.s, vorzugsweise mindestens 0,4 Pa.s, ist.

5. Eine Zusammensetzung nach irgendeinem der vorstehenden Ansprüche, umfassend mindestens 0,4 Gew.-% des Copolymers (ii).

6. Eine Zusammensetzung nach irgendeinem der vorstehenden Ansprüche, wobei das anionische Tensid ausgewählt ist aus der Gruppe, bestehend aus Alkylbenzolsulfonat und Alkylsulfat.

7. Eine Zusammensetzung gemäß irgendeinem der vorstehenden Ansprüche, wobei das anionische Tensid lineares Alkylbenzolsulfonat, Natriumsalz umfasst.

8. Eine Zusammensetzung gemäß irgendeinem der vorstehenden Ansprüche, wobei die Zusammensetzung weiterhin ein Viskositäts-reduzierendes Polymer, ausgewählt aus ethoxyliertem Polyethylenimin und Polyesterschmutzfreisetzendem Polymer enthält.

9. Eine Zusammensetzung gemäß irgendeinem der vorstehenden Ansprüche, wobei das Copolymer (ii) ein Molekulargewicht Mw von mindestens 500.000 Daltons aufweist.

10. Eine Zusammensetzung gemäß irgendeinem der vorstehenden Ansprüche, in der das erste Monomer (A) im Copolymer (ii) Maleinsäureanhydrid ist.

11. Ein Verfahren zur Herstellung einer Reinigungsmittelzusammensetzung, wobei das Verfahren das Mischen eines linearen HASE-Polymers, gebildet aus den Monomeren A, B, C und D, wie vorstehend beschrieben, mit einem Säurevorläufer eines anionischen Tensids umfasst und dann ausreichend Lauge zugegeben wird, um die Tensidsäure zu neutralisieren und das Copolymer zu quellen.

## Revendications

1. Liquide de détergent aqueux épaissi comprenant :
(i) au moins 5 % en masse d'un système de tensioactif comprenant un tensioactif anionique,
(ii) au moins 0,2 % en masse d'un système épaississant comprenant un copolymère linéaire formé par la polymérisation par addition de :
(A) 0,1 à 5 % en masse d'un premier monomère constitué d'un diacide éthyléniquement insaturé de formule (I) :
HOOC-CR₁=CR₂-COOH (I)
ou d'un précurseur d'anhydride cyclique insaturé d'un tel diacide éthyléniquement insaturé, l'anhydride présentant la formule (II) où R₁ et R₂ sont individuellement choisis parmi H, un groupe alkyle en C₁-C₃, phényle, le chlore et le brome ;
(B) 15 à 60 % en masse d'un second monomère monoacide éthyléniquement insaturé constitué d'acide (méth)acrylique ;
(C) 30 à 70 % en masse d'un troisième monomère éthyléniquement insaturé constitué d'un ester alkylique en C₁-C₈ d'acide (méth)acrylique ;
(D) 1 à 25 % en masse, d'un quatrième monomère éthyléniquement insaturé, constitué de Surfmer de formule (III) :
où chaque R₃ et R₄ est à chaque fois indépendamment choisi parmi H, un groupe méthyle, -C(=O)OH, ou -C(=O)OR₅;
R₅ est un groupe alkyle en C₁-C₃₀ ;
Test -CH₂C(=O)O-, -C(=O)O-, -O-, -CH₂O-, -NHC(=O)NH-, -C(=O)NH-, -Ar-(CE₂)_{z}-NHC(=O)O-, -Ar-(CE₂)_{z}-NHC(=O)NH-, ou -CH₂CH₂NHC(=O)- ;
Ar est un groupe aryle divalent ;
E est H ou un groupe méthyle ;
z est égal 0 ou 1 ;
k est un nombre entier dans l'intervalle de 0 à 30 ; et m est égal à 0 ou 1 ; à condition que lorsque k est égal à 0, m est égal à 0, et lorsque k se trouve dans l'intervalle de 1 à 30 ; m est égal à 1 ;
(R₆O)ₙ est un polyoxyalkylène, lequel est un homopolymère, un copolymère statistique, ou un copolymère séquencé d'unités oxyalkylène en C₂-C₄, où R₆ est C₂H₄, C₃H₆, C₄H₈, ou un mélange de ceux-ci, et n est un nombre entier dans l'intervalle de 5 à 250 ; Y est -R₆O-, -R₆-, -C(=O)-, -C(=O)NH-, =R₆NHC(=O)NH-, ou -C(=O)NHC(=O)- ; et
R₇ est un groupe alkyle substitué ou non substitué choisi dans le groupe constitué d'un groupe alkyle linéaire en C₈-C₄₀, alkyle ramifié en C₈-C₄₀, alkyle en C₈-C₄₀ carbocyclique, alkyle en C₂-C₄₀ substitué, phényle, alkyle en C₂-C₄₀ substitué par un groupe aryle, et un ester de complexe en C₈-C₈₀ ; où le groupe alkyle R₇ comprend éventuellement un ou plusieurs substituants choisis dans le groupe constitué d'un groupe hydroxy, alcoxy, et d'un halogène.

2. Composition selon la revendication 1, dans laquelle le quatrième monomère D est un Surfmer avec la formule (IV) : où :
R₈ et R₉ sont chacun indépendamment choisis parmi H, et un groupe alkyle en C₁₋₃ ;
R₁₀ est en C₂-C₄ et des mélanges de ceux-ci, de préférence en C₂;
m, le nombre moyen d'unités alcoxy R₁₀O, est de 6 à 40 ;
R₁₁ est un groupe alkyle ou alkylaryle ou la partie alkyle est linéaire ou ramifiée ; et
le nombre total d'atomes de carbone est de 10 à 40.

3. Composition selon l'une quelconque des revendications précédentes, dans laquelle le quatrième monomère D est un Surfmer avec la formule (V) : où chaque R₈ et R₉ est indépendamment choisi parmi H, un groupe alkyle en C₁ à C₃, de préférence R₈ est un groupe méthyle et R₉ est H, n est compris entre 6 et 40 et m est compris entre 6 et 40, de préférence n est compris entre 10 et 30 et m est compris entre 15 et 35, encore mieux n est compris entre 12 et 22 et m est compris entre 20 et 30.

4. Composition selon l'une quelconque des revendications précédentes, dans laquelle la viscosité du liquide à 20 s⁻¹ et 25°C est d'au moins 0,3 Pa.s, de préférence d'au moins 0,4 Pa.s.

5. Composition selon l'une quelconque des revendications précédentes comprenant au moins 0,4 % en masse du copolymère (ii).

6. Composition selon l'une quelconque des revendications précédentes, dans laquelle le tensioactif anionique est choisi dans le groupe constitué de benzènesulfonate d'alkyle, et de sulfate d'alkyle.

7. Composition selon l'une quelconque des revendications précédentes, dans laquelle le tensioactif anionique comprend un sel de benzènesulfonate d'alkyle linéaire, sodium.

8. Composition selon l'une quelconque des revendications précédentes, dans laquelle la composition comprend de plus un polymère réduisant la viscosité choisi parmi une polyéthylèneimine éthoxylée et un polymère de libération de saleté de polyester.

9. Composition selon l'une quelconque des revendications précédentes, dans laquelle le copolymère (ii) présente une masse moléculaire Mw d'au moins 500 000 Daltons.

10. Composition selon l'une quelconque des revendications précédentes, dans laquelle le premier monomère (A) dans le copolymère (ii) est l'anhydride maléique.

11. Procédé pour la fabrication d'une composition de détergent, le procédé comprenant le mélange d'un copolymère HASE linéaire formé à partir des monomères A, B, C et D comme décrit ci-dessus avec un précurseur d'acide d'un tensioactif anionique et l'addition subséquente d'alcali dans une quantité suffisante pour neutraliser l'acide de tensioactif et gonfler le copolymère.
